

1

2,861,874

## CORROSION INHIBITOR FOR LIGHT PETROLEUM SOLVENTS AND FUELS

Arlie A. O'Kelly, Lewiston, and Clarence A. Weltman, Niagara Falls, N. Y., assignors to Alox Corporation, Niagara Falls, N. Y., a corporation of New York

No Drawing. Application June 23, 1954  
Serial No. 438,852

5 Claims. (Cl. 52—5)

This invention relates to the provision of corrosion inhibitors adapted for use in gasoline, jet fuel (JP#4), and other light petroleum fuels and light petroleum solvents. The entity "JP#4" is a designation, in a U. S. Government Specification MIL-F-5624B, of a low vapor pressure species of "Fuel, Aircraft Turbine, and Jet Engine," which specification is generally restricted to fuels consisting of hydrocarbon compounds of petroleum origin.

The novel corrosion inhibitors of the present invention are designed to be effective in concentrations from 6 to 50 parts per million (p. p. m.) of fuel or solvent, and to protect storage tanks, pipelines, transport vessels and, in general, all equipment for transporting and storing light petroleum products. Since moisture or liquid water is almost always present as contamination from some source, corrosion is normally a serious problem. Storage tanks always "breathe." With changing temperatures over the course of 24 hours, the vapors in a tank expand or contract. When they contract, air is drawn into the tank and the moisture contained in the air may condense. During long tank storage, considerable volumes of water may be introduced, especially during humid weather. The dangers of corrosion in light fuels storage and transport lie in the damage to costly equipment and contamination of the fuel by particles of iron oxide which may scale off the walls of the pipe or tank.

The requirements of a good light fuels inhibitor (LFI) can be summarized as follows:

(a) It shall protect all equipment while in contact with the inhibited fuel and water.

(b) It shall protect metal equipment for short periods after the inhibited fuel is drained from the equipment. Thus, after a tank is drained—or partly drained—the exposed metal surface shall be protected against atmospheric corrosion.

(c) The LFI shall be completely and strongly adsorbed on the metal surfaces it is protecting. In this way the residual protection described under "b" can be effected. This adsorption is also necessary so that equipment can be "treated" by contact with LFI-containing fuels. Subsequent batches of fuel then require less LFI for continued protection of tanks and equipment. Subsequent lots of fuel may require only 6–10 p. p. m. for continued protection because the metal already has an adsorbed film of inhibitor.

(d) A further manifestation of "b" and "c" above occurs in sea-going tankers. The tanker may deliver a load of fuel and then fill the tanks with salt water as ballast for the return trip. The use of inhibited fuel greatly reduces corrosion difficulties on the return trip. Corrosion is not completely eliminated by the thin adsorbed film of LFI.

(e) The LFI shall not increase gumming tendency or oxidation tendency of the fuel.

It shall be compatible performance-wise with metal

2

deactivators anti-oxidants, TEL, or other additives normally used in the fuels.

It has been found that a light fuels inhibitor, meeting the above criteria, can be produced by admixing a major amount of polymerized linoleic acid—hereinbelow more specifically described—with a minor but effective amount of an oil-soluble dimethyl dialkyl ammonium chloride having the formula:

10



wherein each R represents an alkyl group having from 15 8 to 18 carbon atoms.

Preferably the quaternary ammonium salt used is a product, sold under the trade-name "Arquad 2C," of which the alkyl groups are composed of a mixture of the following:

20

|                               | Percent |
|-------------------------------|---------|
| Octyl (C <sub>8</sub> )       | 8       |
| Decyl (C <sub>10</sub> )      | 9       |
| Dodecyl (C <sub>12</sub> )    | 47      |
| Tetradecyl (C <sub>14</sub> ) | 18      |
| Hexadecyl (C <sub>16</sub> )  | 8       |
| Octadecyl (C <sub>18</sub> )  | 10      |

the trade product being a 50% solution of the salt in isopropanol.

30

The polymerized linoleic acid component of the present corrosion inhibiting composition is a product, variously known as "dimer acid" and "dilinoleic acid," produced by polymerizing linoleic acid under conditions to yield approximately 85% of the dimer, approximately 12% of the trimer, and only a few, e. g., 3%, of unpolymerized monomer. The preferred polymerized linoleic acid component of the present composition is one sold under the trade designation "Empol 1022," having the following significant properties:

40

|                           |                                                                              |
|---------------------------|------------------------------------------------------------------------------|
| Iodine value              | 80–95                                                                        |
| Acid value                | 180–192                                                                      |
| Saponification value      | 185–195                                                                      |
| Neutralization equivalent | 290–310                                                                      |
| Solubility                | Insoluble in water; soluble in Stoddard Solvent, oils, waxes, resins, fuels. |

Preferably the composition of the present invention 50 is composed essentially of approximately 10–90% by weight of the polymerized linoleic acid and approximately 90–10% of the dimethyl dialkyl ammonium chloride (50% active in isopropanol). The composition may, and preferably does, include also a suitable amount of a petroleum solvent or oil to impart a desirable fluidity 55 to the composition for ease of handling and "dosage": this latter ingredient is not, however, an essential part of the composition.

It has been discovered that the composition of the 60 present invention affords a striking illustration of synergistic effect—as more particularly will be brought out in the hereinbelow portions of this disclosure sub-titled "Table I" and "Table II"—in that essentially any combination of (a) polymerized linoleic acid and (b) dimethyl dialkyl ammonium chloride is exceedingly more effective as a light fuels inhibitor than is either (a) or (b) alone. A ratio of 90% "Empol 1022" to 10% "Arquad 2C" is preferred because it combines outstanding effectiveness with economy. Increasing the ratio of "Arquad 2C" beyond about 10% materially increases the cost of the additive without material improvement in

the effectiveness of the composition. With 40 parts by weight of this mixture there may be included from about 40 to about 80 parts, preferably 60 parts, by weight of Stoddard Solvent or other hydrocarbon solvent as fluidizing agent or "carrier."

The effectiveness of the above-described light fuels inhibitor was established by the following experimental work:

#### A. TEST METHOD

(1) The test method used to evaluate light fuels inhibitors was ASTM-D-665-49T. However, our tests were run at a temperature of 80° F. The ASTM method calls for 140° F. In this test, a polished steel rod is immersed in a beaker containing 300 ml. of inhibited fuel and 30 ml. of synthetic sea water. The mixture is stirred rapidly so that the oil and sea water flow over the test rod. The length of time the test is run is arbitrary. We have selected 24 hours as prescribed in ASTM D-665.

The test rod is examined periodically for visual signs of rust. When 5-10% of the surface is rusted we have recorded it as a failure. Any product noted as a "pass" shows no corrosion after 24 hours of exposure to the rapidly stirred fuel-sea water mixture.

(2) To determine residual rust protection, a complete test, as described above, was run. After 24 hours, the inhibited fuel was removed from the beaker and replaced by 300 ml. of uninhibited fuel. Additional sea water was also added. Stirring was continued until failure of the specimen.

#### B. FUELS SELECTED

Most of the development work concentrated on three fuels:

- (1) 36/40 Bé. distillate. Kerosene.
- (2) High test gasoline.
- (3) Jet fuel. JP #4 (procured from U. S. Air Force).

#### C. PROCEDURE

All test work was based on combinations of Empol 1022 and Arquad 2C as the active components.

To prepare solutions at very low concentrations of additive, "concentrates" containing 1% additive in a light petroleum solvent (Varsol) were used. The following summary shows the amounts of "Concentrate" used:

2 g. of (1% additive in Varsol) + 398 g. fuel = 0.005% additive in fuel (50 p. p. m.)  
 1 g. of (1% additive in Varsol) + 399 g. fuel = 0.0025% additive in fuel (25 p. p. m.)  
 0.5 g. of (1% additive in Varsol) + 399.5 g. fuel = 0.0012% additive in fuel (12 p. p. m.)  
 0.5 g. of (1% additive in Varsol) + 799.5 g. fuel = 0.0006% additive in fuel (6 p. p. m.)

350 ml. of test fuel were added to the beaker. The test rod, stirrer and thermometer were assembled, and stirring started. After 30 minutes of stirring, 50 ml. of fuel were removed by pipette, and 30 ml. of sea water added. The time of addition of sea water is taken as the time of starting the test.

#### D. RESULTS

The results for jet fuels are summarized in Table I. The results for hi-test gasoline are summarized in Table II.

The results for kerosene are not summarized because they are similar in magnitude to those for gasoline.

Table III presents selected data demonstrating residual rust protection.

Table IV summarizes the effects of a high concentration of LFI in gasoline on the standard gum determinations.

4  
Table I

[ASTM-D-665-49T. Results for inhibited JP4 jet fuels.]

| 5  | Additive Composition                                    | Percent composition in JP4 | p. p. m. composition in JP4 | ASTM-D-665 Result        | Time (Hrs.)    |
|----|---------------------------------------------------------|----------------------------|-----------------------------|--------------------------|----------------|
| 10 | (a) Empol 1022                                          | 0.0025<br>0.005            | 25<br>50                    | Fail*<br>Pass            | 16<br>24       |
|    | (b) A mixture of 10% Arquad 2C (50%) and 90% Empol 1022 | 0.0006<br>0.0012<br>0.0025 | 6<br>12<br>25               | 5% Rust<br>Pass<br>Pass  | 20<br>24<br>24 |
|    | (c) A mixture of 30% Arquad 2C (50%) and 70% Empol 1022 | 0.0006<br>0.0012<br>0.0025 | 6<br>12<br>25               | 10% Rust<br>Pass<br>Pass | 20<br>24<br>24 |
| 15 | (d) A mixture of 50% Arquad 2C (50%) and 50% Empol 1022 | 0.0012<br>0.0025           | 12<br>25                    | 25% Rust<br>Pass         | 24<br>24       |
|    | (e) A mixture of 70% Arquad 2C (50%) and 30% Empol 1022 | 0.0006<br>0.0012           | 6<br>12                     | 20% Rust<br>Pass         | 20<br>24       |
|    | (f) A mixture of 90% Arquad 2C (50%) and 10% Empol 1022 | 0.0012<br>0.0025           | 12<br>25                    | 25% Rust<br>Pass         | 17<br>24       |
| 20 | (g) Arquad 2C (50%)                                     | 0.005                      | 50                          | 50% Rust<br>100% Rust    | 4<br>2         |
|    | None                                                    |                            |                             |                          |                |

\*40% rust after 16 hrs.

Table II

[ASTM-D-665-49T. Results for inhibited hi-test gasoline.]

| 25 | Additive Composition                                    | Percent composition in Gasoline | p. p. m. composition in Gasoline | Result           | Time (Hrs.) |
|----|---------------------------------------------------------|---------------------------------|----------------------------------|------------------|-------------|
| 30 | (a) Empol 1022                                          | 0.0025<br>0.005                 | 25<br>50                         | 5% Rust<br>Pass  | 24<br>24    |
|    | (b) A mixture of 10% Arquad 2C (50%) and 90% Empol 1022 | 0.0006<br>0.0012                | 6<br>12                          | Pass<br>Pass     | 24<br>24    |
|    | (c) A mixture of 30% Arquad 2C (50%) and 70% Empol 1022 | 0.0006<br>0.0012                | 6<br>12                          | Pass<br>Pass     | 24<br>24    |
| 35 | (d) A mixture of 50% Arquad 2C (50%) and 50% Empol 1022 | 0.0006<br>0.0012                | 6<br>12                          | 30% Rust<br>Pass | 24<br>24    |
|    | (e) A mixture of 70% Arquad 2C (50%) and 30% Empol 1022 | 0.0006<br>0.0012                | 6<br>12                          | Pass<br>Pass     | 24<br>24    |
| 40 | (f) A mixture of 90% Arquad 2C (50%) and 10% Empol 1022 | 0.0012<br>0.0025                | 12<br>25                         | 20% Rust<br>Pass | 24<br>24    |
|    | (g) Arquad 2C (50%)                                     | 0.005                           | 50                               | 40% Rust         | 4           |

Table III

#### RESIDUAL RUST PROTECTION

[In ASTM D-665-49T rust test.]

| 50 | Composition                                        | Percent in Gasoline        | After addition of uninhibited gasoline |             |
|----|----------------------------------------------------|----------------------------|----------------------------------------|-------------|
|    |                                                    |                            | Result                                 | Time, hours |
| 55 | Empol 1022                                         | 0.0025                     | 50% Rust                               | 3           |
|    | Arquad 2C (50%)                                    | 0.0025                     | do                                     | 2           |
|    | A mixture of 90-Empol 1022 and 10-Arquad 2C (50%). | 0.0006<br>0.0012<br>0.0025 | 30% Rust<br>do<br>20% Rust             | 4<br>6<br>8 |

Table IV

#### EFFECT OF LFI ON GUM DETERMINATIONS IN GASOLINE

| 65 | Fuel Mixture               | Copper Dish Gum (mg./100 ml.) | ASTM D-873-49 Potential Gum (mg./100 ml.) | ASTM D-881-49 Existent Gum (mg./100 ml.) |
|----|----------------------------|-------------------------------|-------------------------------------------|------------------------------------------|
| 70 | Hi-Test Gasoline (Blank)   | 9.0                           | 9.0                                       | 3.0                                      |
|    | Hi-Test Gasoline 0.01% LFI | 16.0                          | 12.0                                      | 6.0                                      |

We claim:

1. A corrosion inhibitor composition for use in JP4 jet fuels and hi-test gasoline, said composition consisting essentially of a mixture of from about 90 to 70% by weight of polymerized linoleic acid and from about

10 to about 30% by weight of an oil-soluble dimethyl dialkyl ammonium chloride of the formula



5

in which each R represents an alkyl group having from 8 to 18 carbon atoms.

2. The composition defined in claim 1, in which the mixture is dissolved in a light solvent of petroleum origin 10 as fluidizing agent.

3. The composition defined in claim 1, in which the mixture contains 10 percent by weight of said dimethyl dialkyl ammonium chloride and 90 percent by weight of said polymerized linoleic acid.

4. A solution consisting essentially of about 40% by weight of the composition defined in claim 1 in about 60% by weight of Stoddard Solvent.

5. An inhibited light petroleum fuel of the group consisting of JP4 jet fuels and hi-test gasoline containing a 20 corrosion inhibitor composition consisting essentially of a mixture of from about 90 to about 70% by weight of polymerized linoleic acid and from about 10 to about

30% by weight of an oil-soluble dimethyl dialkyl ammonium chloride of the formula



wherein each R represents an alkyl group having from 8 to 18 carbon atoms, said corrosion inhibitor composition being present in said fuel in an amount upwards from 12 p. p. m. in the case of a JP4 jet fuel and in an amount upwards from 6 p. p. m. in the case of a hi-test gasoline.

References Cited in the file of this patent

UNITED STATES PATENTS

- |           |                     |               |
|-----------|---------------------|---------------|
| 2,632,695 | Landis et al. ----- | Mar. 24, 1953 |
| 2,659,693 | Lytle -----         | Nov. 17, 1953 |
| 2,676,987 | Lewis et al. -----  | Apr. 27, 1954 |

OTHER REFERENCES

- Baker et al.: Ind. and Eng. Chem., vol. 41, No. 1, January 1949, pp. 137-144.